

T. J. CLARK,

BEATER BAR.

APPLICATION FILED JAN. 9, 1920.

1,378,167.

Patented May 17, 1921.



FIG. 2.



FIG. 3.



FIG. 4



INVENTOR

TERRENCE J. CLARK

By Joseph J. O'Brien  
ATTORNEY

# UNITED STATES PATENT OFFICE.

TERRENCE J. CLARK, OF HOLYOKE, MASSACHUSETTS.

## BEATER-BAR.

1,378,167.

Specification of Letters Patent. Patented May 17, 1921.

Application filed January 9, 1920. Serial No. 350,461.

To all whom it may concern:

Be it known that I, TERRENCE J. CLARK, a subject of the King of England, residing at Holyoke, in the county of Hampden and 5 State of Massachusetts, have invented certain new and useful Improvements in Beater-Bars, of which the following is a specification.

This invention relates to improvements 10 in bars for beating engines used in the beating up of pulp and stock for the making of paper and its leading object is to provide a bar which will have a cutting edge of hardened steel and a core of steel and relatively 15 thick coats on its sides composed of a high grade iron, which will offer greater resistance to corrosion from the action of the acids used in paper making than steel offers.

Another object of the invention is to provide 20 a composite bar of this type which will resist fracture due to continued use and to minimize the tendency of the steel to crystallize.

With the above and other objects in view 25 this invention relates to certain new and useful constructions, combinations and arrangements of parts, clearly described in the following specification and fully illustrated in the accompanying drawings, in 30 which:

Figure 1 is a transverse sectional view of my improved beater bar.

Fig. 2 is a bottom plan view thereof.

Fig. 3 is a top plan view thereof.

Fig. 4 is a side elevation showing the 35 working edge of the bar.

Referring to the accompanying drawings A designates a composite beater bar which consists of a steel core B and iron coat C welded to one side of the core B and an iron coat D welded to the opposite side of the core D. The coats C and D are welded to the core B under the action of a trip hammer

or by any other method that may be desired. One edge portion of the core B is deflected 45 laterally to provide a cutting edge E, which is hardened and which constitutes the working edge of the beater bar for cutting up the stock in the beater engine. The coat C thus covers practically all of one side of the 50 bar, excepting the deflected portion or edge E while the coat D covers the entire opposite side of the bar and is deflected at F so as to reinforce the portion of the steel core D which is deflected to provide the working 55 or cutting edge. The coat D is preferably thickened longitudinally at d so as to reinforce the central portion of the bar.

By the construction of my beater bar a 60 steel center of great strength can be employed which will provide a durable working edge, while the side faces of the bar are protected against excessive corrosion by the use of relatively thick coats of high grade iron, which has greater resistance than steel 65 to the corrosion of the acids used in the digestion of the raw stock employed in paper making.

Having described my invention, I claim:

1. A beater bar having a steel center and 70 a coat of iron welded to each side thereof, one edge portion of the steel center being deflected toward the side of the bar to provide a steel cutting edge.

2. A beater bar consisting of a steel center 75 having a portion deflected to the side thereof to provide a cutting edge, a coat of iron welded to one side of said center and having its outer face substantially flush with the deflected portion of said center, and a second 80 coat of iron welded to the opposite side of the center and covering the deflected portion of said center.

Signed by me at Springfield, Mass.

TERRENCE J. CLARK.